

## UNITED STATES PATENT OFFICE

MERRILL M. THOMPSON AND JAMES C. PATTEN, OF INDIANAPOLIS, INDIANA; SAID THOMPSON ASSIGNOR TO SAID PATTEN; MARGARET LUCILE PATTEN EXECUTRIX OF SAID JAMES C. PATTEN, DECEASED

## PLATING ZINC-TIN ALLOY

No Drawing.

Application filed September 2, 1930. Serial No. 479,414.

This invention relates to plating zinc-tin alloys; and it comprises an improvement in methods of electrically depositing zinc-tin alloy coatings upon iron, steel and other metals wherein soluble anodes of zinc-tin alloys are used and these anodes are amalgamated with mercury, the plating solution being usually alkaline and usually containing a substantial amount of sulfonated castor oil (Turkey red oil); all as more fully herein-after set forth and as claimed.

The protection against corrosion afforded to iron and steel by an electroplated coating depends partly upon its continuity and partly upon the position of the coating metal in the electrochemical scale. Copper coatings, for example, owe their entire value to their continuity, since copper is electronegative to iron and, with a break or pore in the coating, corrosion is accelerated. Zinc, being highly electropositive to iron, protects not only because of its shielding value, but because corrosion is restricted to zinc where both zinc and iron are exposed. However, this also means that the zinc corrodes more quickly because of the presence of iron; any kind of pore or break in the surface tending to enlarge. Cadmium coatings have lately come into extensive use, since, in addition to their decorative value, they are found in practice to have great protective value even with very thin films; a fact which is probably due, in part, to the position of cadmium relative to iron in the electrochemical scale. It does not tend to accelerate corrosion of the iron. Cadmium coatings have a much greater protective value than zinc coatings. Standard salt spray tests on electrodeposited zinc coatings on iron or steel sheets indicate an average life of about 200 hours with a coating of about 0.0012 inches, while much thinner cadmium coatings, say, only 0.0002 inches will give a life of 500 to 1,000 hours. A cadmium coating on iron of 0.0003 inches is sometimes regarded as equivalent, for protective purposes, to a zinc coating of 0.001 inches.

Cadmium is, however, a relatively expensive metal; much more expensive than zinc. It is a desirable object in the art to provide a coating better than one of zinc and less expen-

sive than one of cadmium. In another and copending application Ser. No. 433,500, on which the present invention is in some aspects an improvement, this object is obtained by providing iron and steel with an electrically deposited coating of an alloy of zinc and tin. The ratio of zinc to tin may vary between 93:7 and 65:35. The particular ratio depends upon the properties desired in the coating. Deposition is from an equi-potential bath of alkaline character containing a pyrophosphate and a cyanide. An equi-potential bath is one in which electrically connected bars of tin and zinc show development of no substantial potential. Replenishment of the bath may be by alloy anodes or by pairs of zinc and tin anodes having the desired ratio of surface.

The appearance of articles electrically coated with zinc-tin alloys is extremely decorative. They can be readily buffed and polished. The protection given the underlying metal in case of iron and steel is of the same order as that afforded by cadmium. The coating is advantageous on other metals than iron and steel, as upon copper and brass. The coating is an excellent base for deposition of chromium or of nickel, serving for this purpose like the cadmium of Patent No. 1,615,585.

In electrical deposition of these alloys, it has been found useful to amalgamate the soluble anodes used, thus promoting the desired proportioned solution of the two metals, zinc and tin. Amalgamation also reduces non-electric attack of the bath on the anode. As these baths are customarily quite alkaline, this is desirable. Both zinc and tin being soluble in mercury, it is probable that in the use of the amalgamated alloy anodes the zinc and tin passing into solution in the bath as an intermediate phase go into solution in the mercury; that the active anode is really a mercury solution of the two metals.

With the use of amalgamated alloy anodes, it is found that the equi-potential character of the bath is of less importance and that ordinary salines may be used; ordinary salts such as zinc sulfate and stannous chloride being dissolved in a solution of caustic soda.

With any alkaline bath for the deposition of zinc-tin alloys, it is found that the presence of an "addition agent" is of advantage. The best of these addition agents, so far as is at present known, is sulfonated or sulfated 5 castor oil or ordinary commercial Turkey red oil. In making Turkey red oil, other oils than castor oil may be employed. Sulfonated mineral oils and sulfonated aromatic compounds may be used for the present purposes. 10 Where the sulfonated preparations are acid, they react with the bath and it is necessary to use enough alkali to redissolve any precipitate which they may form.

While, as stated, zinc-tin alloys with widely varying ratios may be deposited and are desirable for various purposes, the ratio varying from perhaps 93:7 to 65:35, it has been found that in using the present invention a 20 ratio of 90:10 or thereabouts, is most desirable. With a zinc-tin coating alloy containing 10 per cent tin, the properties are quite like those of cadmium, but the coating is, in some respects, better than that produced with 25 cadmium. It is considerably cheaper and serves better as a base layer for chrome plating and for nickel plating.

In a specific embodiment of the present invention producing a 10 liter bath containing 30 dissolved zinc and tin in the 90:10 ratio desired, 810 grams of commercial crystallized zinc sulfate ( $ZnSO_4 \cdot 7H_2O$ ) are dissolved in water and 35 grams of commercial stannous chloride ( $SnCl_2 \cdot 2H_2O$ ) are dissolved in 35 water. The solutions are mixed and to the mixture is added a solution of 1500 grams of commercial sodium hydroxide. Enough water is then added to make the volume 10 liters. A white precipitate is formed at first on the 40 addition of the alkali solution, but this quickly redissolves. To the 10 liter bath thus formed is next added 100 cc. of commercial liquid Turkey red oil. From this bath a coating of 45 alloy in the 90:10 ratio may be deposited and by the use of alloy anodes having the same ratio, the character of the bath remains unchanged over long periods of time.

The anodes used in the present invention are prepared by melting together the desired 50 amounts of zinc and tin in the ratio of 90:10. The molten alloy is cast into a suitable mold. For amalgamation the cast anodes thus produced are immersed in a slightly acid solution of mercurous or mercuric nitrate. The 55 amount of dissolved mercury should be equal to about 2 per cent of the weight of the anodes. The anodes are left in the mercury solution for several hours or until the solution is stripped of mercury. The anodes may be 60 left in the solution over night. Amalgamated anodes made as described give good results in any sufficiently alkaline bath, dissolving only when the current is on and giving up to the bath zinc and tin in the ratio in which they 65 are contained in the alloy. They afford good

coatings. The Turkey red oil in the solution is an efficient addition agent and much promotes deposition of compact reguline metal. The cathode efficiency varies between 90 and 95 per cent. For ordinary thicknesses 70 of coating using a current density of 10 to 20 amperes per square foot at 6 volts, about 30 minutes plating time will give a coating 0.0002 to 0.0004 inches thick which is sufficient for all ordinary purposes. On such a coating, 75 after buffing and polishing, an impervious chromium or nickel coating may be deposited by the ordinary coating methods.

The throwing power of a bath under the present invention is unusually good. The 80 coatings formed are uniform, flawless and poreless. As regards protecting the underlying metal they are better than those by the electrolytic deposition of zinc from the standard baths; and stand up better. For example where a zinc coating of 0.0003 inches on Armco iron will stand up under a salt spray for about 100 hours, a similar thickness of coating of zinc-tin alloy will stand up about 85 1000 hours under the same conditions.

What we claim is:

1. In the electroplating of iron and steel articles with a protective coating of alloy, the process which comprises passing current 95 between anodes and the said articles serving as cathodes, said cathodes and anodes being immersed in a bath containing zinc and tin in solution and said anodes being a zinc-tin alloy amalgamated with mercury.

2. In the electroplating of iron and steel articles with a zinc-tin alloy the process which comprises passing current through a 100 bath containing zinc and tin in solution and between a plurality of anodes and the said articles serving as cathodes, the said anodes being a zinc-tin alloy amalgamated with mercury.

3. In the electroplating of iron and steel articles with a zinc-tin alloy the process which comprises passing an electric current 110 through a solution comprising zinc and tin in solution and a sulfonated oil, between anodes and said articles serving as cathodes, the said anodes comprising a zinc-tin alloy 115 amalgamated with mercury.

4. In the electroplating of iron and steel articles with a zinc-tin alloy the process which comprises passing an electric current through an alkaline solution comprising zinc sulfate and stannous chloride in solution and 120 a sulfonated castor oil, between anodes and the said articles serving as cathodes, the said anodes comprising a zinc-tin alloy amalgamated with mercury.

5. In the electroplating of iron and steel 125 articles with zinc-tin alloys at predetermined metallic ratios, the process which comprises passing current through a bath between anodes and the said articles serving as cathodes, the said bath containing zinc and tin 130

in approximately said predetermined ratio, and the said anode being a zinc-tin alloy amalgamated with mercury, the zinc and tin of said alloy being in a ratio of 90:10.

5 6. In the electroplating of iron and steel articles with zinc-tin alloys at predetermined metallic ratios, the process which comprises passing current through a bath between anodes and the said articles serving as cathodes, the said bath containing zinc and tin in approximately said predetermined ratio, and the said anode being a zinc-tin alloy amalgamated with mercury, the zinc and tin of said alloy being in a ratio of 90:10 and the 10 amount of mercury being about 2 per cent of the alloy.

15 7. As a new anode suitable for electroplating iron and steel articles with zinc-tin alloys, an anode comprising a zinc-tin alloy amalgamated with mercury.

20 8. As a new anode suitable for electroplating iron and steel articles with zinc-tin alloys, an anode comprising a zinc-tin alloy amalgamated with mercury, the zinc and tin 25 of said alloy being in the ratio of 90:10.

30 9. As a new anode suitable for electroplating iron and steel articles with zinc-tin alloys, an anode comprising a zinc-tin alloy amalgamated with mercury, the zinc and tin 35 of said alloy being in the ratio of 90:10 and the amount of mercury being about 2 per cent of the alloy.

In testimony whereof, we have hereunto affixed our signatures.

35 MERRILL M. THOMPSON.  
JAMES C. PATTEN.

40

45

50

55

60

65